

(No Model.)

C. H. WILDER

MOL. D.

No. 404,372.

Patented May 28, 1889.



Fig. 1.



Fig. 2.

Witnessed:  
C.W. Houghtaling  
Frank Bean

Inventor.  
Charles H. Wilder

# UNITED STATES PATENT OFFICE.

CHARLES H. WILDER, OF NATICK, ASSIGNEE, BY MESNE ASSIGNMENTS, TO  
FREDERICK E. ATTEAUX, TRUSTEE, OF BOSTON, MASSACHUSETTS.

## MOLD.

SPECIFICATION forming part of Letters Patent No. 404,372, dated May 28, 1889.

Application filed May 4, 1888. Serial No. 273,002. (No model.)

*To all whom it may concern:*

Be it known that I, CHARLES H. WILDER, of Natick, in the county of Middlesex and State of Massachusetts, a citizen of the United States, 5 have invented certain new and useful Improvements in the Manufacture of Molds for Metallic Castings, of which the following is a specification.

My invention relates to an improvement in the formation of molds from which to cast metal articles, and its object is to produce a mold such that its inner or molding-surface will not be in any degree fused or fluxed by the contact of the molten metal, but will at all 15 times have and preserve a smooth and indestructible molding-face, whereby not only can more perfect castings be obtained than has heretofore been possible, but also the same mold may be repeatedly used for producing 20 castings.

My invention also includes a convenient form in which the mold can be made and thereby preserved against accidental injury in handling, all as will be hereinafter more 25 fully set forth and explained.

For the further explanation of my invention I have shown in the accompanying drawings at Figure 1, one part of a flask and one part of a mold for a cylindrical casting, and 30 a cylinder of cast metal in the mold, part of the casting which would be formed in the other part of the mold being above the surface in the part of the mold shown. Fig. 2 shows a transverse section on the line 2 2 of Fig. 1 35 of the flask, mold, and casting.

The outer wall of flask is marked  $a$ , the mold is marked  $a'$ , and the casting is marked  $a''$ .

The mold is represented in the drawings as composed of two parts, the inner portion,  $a^3$ , 40 being formed of my improved mold material, and the outer portion of a strengthening or protecting material, as will be hereinafter explained. A layer of sand is represented at  $a^4$  between the mold and the outer wall of the flask. The customary dowels and sockets for joining adjacent portions of the mold are represented at  $a^5$ , and flanges  $a^6$  are provided on the edges of the flask to retain the sand between the mold and flask.

50 My improved mold is formed of a mixture of pulverized coke and pulverized graphite;

or, as it is commercially known, "plumbago." In preparing this mixture I grind each of the substances to as fine a powder as is readily practicable, the graphite, as is well known, 55 being capable of a considerably finer reduction than the coke. After the two substances have been thus ground I unite or incorporate them with each other mechanically in any convenient manner. The function of the coke 60 in the mixture thus formed is that which comes from its refractory and infusible character. The function of the graphite is through its equally refractory character and through its much greater fineness of grain to fully permeate and fill up the interstices that would otherwise occur among the grains of coke, thus giving to the mixture as a whole a much more compact texture or grain, and consequently much greater capacity for exactly 65 preserving and reproducing the form of the article to be cast than would be possible if coke alone were employed.

The mixture of coke and graphite above described may be used in the same manner as 70 common molding-sand is now employed, and forms the subject-matter of another application for patent. Inasmuch, however, as a mold, if made in the ordinary manner by a pattern in a loose mixture such as has been 75 described, is readily disturbed and destroyed by handling, I prefer in using my improved mixture for molding to give to the mold a permanent form. This I do by mixing with a suitable portion of the coke and graphite mixture 80 a suitable plastic cokable binder—such as melted pitch or tar—in sufficient proportion to make the whole mass plastic. The plastic mass thus obtained may be pressed or tamped around the article or pattern duplicates of 85 which the mold is intended to produce. When the interior face of the mold has thus been given the desired form and after it has cooled, in order to make it permanent and convenient for repeated handling, I place the mold within 90 a suitable metal box or case and surround it therein with sand. This box is then closed, placed in a heating-furnace, and subjected to heat at a temperature and for a period sufficient to convert the binder into coke. The 95 mold then, after being allowed to cool, may be repeatedly used in the ordinary manner to 100

furnish castings of the form originally impressed upon it, as before explained. The permanent or portable mold thus obtained will sometimes, however, be found to lack the 5 strength required to withstand the handling to which it may be subjected; therefore, to meet this defect, I may provide it with an exterior or backing, as I will now proceed to describe.

10 After the mixture of coke, graphite, and the binder has been pressed or tamped upon the pattern I take a sufficient quantity of pulverized coke and mix it with an adhesive cokable binder, thus forming a second plastic 15 mass; and this second mass I spread over the back or outer portion of the mold formed of coke and graphite bound together, and temporarily unite the two under moderate pressure while the mass of the backing is 20 still plastic. I then place the combined mold and backing in a sand-filled case and subject the whole to the coking operation in a furnace, as before described, continuing this until the whole of the binder throughout the 25 mass has been converted to coke, thereby producing a mold formed of a mixture of coke

and graphite, and a backing for the mold formed of coke, the whole integrally united.

It will be understood that a mold so formed will be used in casting in the ordinary manner, the molds being made sectional and provided with dowels and sockets or other well-known appropriate devices for uniting them in readiness for casting, and a flask and sand filling being applied in the usual manner. 30 35

I claim—

1. As a new article of manufacture a permanent mold formed of coke, graphite, and a coked binder, as described.

2. As a new article of manufacture, a permanent mold provided with an integrally-attached back, the face of the said mold being formed of a mixture of coke, graphite, and coked binder, all substantially as described, and the backing of said mold being 40 45 formed of coke and a coked binder, the said mold and back being united, substantially as set forth.

CHARLES H. WILDER.

Witnesses:

CHS. HOUGHTON,  
WM. E. PEABODY.